

## UNITED STATES PATENT OFFICE

2,280,118

## PROCESS OF SULPHONATION

Bernard A. Dombrow, New York, N. Y., assignor to National Oil Products Company, Harrison, N. J., a corporation of New Jersey

No Drawing. Application February 10, 1938,  
Serial No. 189,892

14 Claims. (Cl. 260—400)

The invention relates, in general, to sulphonated fatty materials and, in particular, to an improved process for producing sulphonated fatty oils and waxes and to correlated improvements in the products thus produced.

According to the usual procedure in producing sulphonated fatty oils and waxes, the fatty material is subjected to sulphonation with any suitable sulphonating agent such as sulphuric acid, chlorsulphonic acid,  $SO_3$ , etc. The quantity of  $SO_3$  organically combined with the fatty oil or wax may usually be varied within certain limits depending upon the particular method employed and depending further upon the conditions maintained during sulphonation. In any event, however, the sulphonated products derived from the conventional processes contain not more than about 10% organically combined  $SO_3$  and in most cases the  $SO_3$  content lies within the range of about 4% to 9%. While these ordinary sulphonated fatty oils and waxes have found extensive use in many fields, they are characterized by being unstable under certain conditions. They tend to separate and decompose on standing or in the presence of aqueous acid or salt solutions, thereby resulting in a sludge formation. Where such sulphonated products are used in textile treatments, for example, the separation and decomposition lead to spotting or staining of the fibers.

The general object of the present invention is to obviate the foregoing and other disadvantages.

A specific object of the invention is to provide improved sulphonated fatty oils and waxes having an enhanced stability when subjected to normal use.

Another object of the invention is to provide improved sulphonated fatty oil and waxes which are substantially resistant to decomposition in the presence of acid or salt solutions.

A further object of the invention is to provide an improved process of producing highly stable sulphonated fatty oils and waxes.

Other objects of the invention will in part be obvious and will in part appear hereinafter.

It has been found that the stability of sulphonated fatty oils and waxes may be greatly improved by increasing the organically combined  $SO_3$  content to a value above 10%. Such products are also particularly resistant to the formation of sludge or the separation of greasy or fatty deposits upon standing or in the presence of acids or salts. These products of increased  $SO_3$  content are not, however, readily produced by direct sulphonation.

In order to obtain highly sulphonated products it has even been proposed in some instances to oxidize and hydroxylate the aliphatic chains of the high molecular weight fatty materials to provide more places for attachment of  $SO_3$  groups and thus enable the compounds to be sulphonated to a higher degree, but these oxidation and hydroxylation methods do not produce high yields of the desired materials. In any case, it is not readily possible directly to increase the  $SO_3$  content of these fatty materials to above 10% without extended and difficult procedures involving substantial increased cost in raw materials and more expensive apparatus with decreased yields of the desired sulphonated product.

It appears that the usual sulphonated fatty oils or waxes containing less than 10% of  $SO_3$  contain substantial quantities of unsulphonated materials which tend to give rise to the instability of the products. It further appears that when these unsulphonated materials are partly removed to give a product of increased  $SO_3$  content, the stability of the sulphonated material will be greatly enhanced.

According to the invention, the process comprises subjecting a sulphonated fatty oil or wax to agitation with a water-miscible aliphatic organic solvent. After admixture of the solvent and sulfonated product two distinct layers are formed upon standing, the upper layer containing the solvent and high  $SO_3$  fraction and the lower layer containing the lower  $SO_3$  fraction. The solvent employed must be miscible with the sulphonated fraction and substantially immiscible with the unsulphonated fraction in the presence of each other and moisture. The acid value of the sulphonated product may be adjusted according to the particular solvent to be employed. In the use of a solvent such as acetone or acetone alcohol, better results are obtained if a product of a low acid value is used whereas a product of a relatively higher acid value is more suitable when a solvent such as mesityl oxide is employed. The relationship between any suitable solvent with respect to the acid value of the sulphonated product may be readily ascertained by the trial and error method.

The invention accordingly comprises the several steps and the relation of one or more of such steps with respect to each of the others, and the product possessing the features and properties, which are exemplified in the following detailed disclosure, and the scope of the invention will be indicated in the claims.

The process of the invention is directed particularly to the treatment of sulphonated fatty oils and waxes, a few examples of which may be given as follows: castor oil, olive oil, neat's-foot oil, cottonseed oil, rapeseed oil, corn oil, cod oil, fish oils in general, tallow, sperm oil, etc.

Any suitable water-miscible, aliphatic organic solvent or mixture of the such solvents, may be used, such for example, as ketones, such as acetone, ethyl propyl ketone, mesityl oxide, etc., alcohols, such as methyl, ethyl, isopropyl etc., ethers, such as dioxane, amines, such as trimethylamine, ketone-alcohols, such as diacetone-alcohol, etc. Solvents such as methanol, ethanol and acetone are preferred in view of their efficient extraction, ease of handling, low cost, etc. A relatively small amount of water may be used with the solvent but in most cases addition of water will not be necessary as the quantity of water normally present in the sulphonated product will be sufficient to insure proper separation of the fractions. The amount of solvent used may be varied to obtain the desired results. The ratio of solvent to be used depends upon the extraction or split desired. The less solvent employed, the higher the SO<sub>3</sub> content of the oil extracted, but the lower the yield of high SO<sub>3</sub> material. In other words, the SO<sub>3</sub> content of the extracted product is inversely proportional to the yield obtained. This relationship will be more fully described hereinafter.

In carrying out the process, the solvent is preferably used in amounts equal to or greater than that of sulphonated fatty oil or wax to be treated. After thorough agitation of the solvent and sulphonated material, the mixture is allowed to settle whereupon two layers will be formed, one layer containing most of the solvent and the sulfonated product of increased SO<sub>3</sub> content and the other layer containing the unsulphonated or sulphonated material of low SO<sub>3</sub> content. The extraction may be repeated several times if desired. The temperature under which the extraction step is carried out may be varied within wide limits, it being highly preferable, however, to carry out this step within a range between room temperature to 0° C. or lower. After separation of the layers, they may be subjected to distillation to drive off the solvent which may be recovered for subsequent use. The fraction bearing the unsulphonated or low SO<sub>3</sub> products may be used as such or they may be utilized as raw material for further sulphonation.

While use of the terms "extracting" and "extraction" has been made herein with respect to the separation of the fractions containing high and low SO<sub>3</sub> contents, these terms are not used according to their usual meaning inasmuch as the action of the solvent is not essentially one of extraction but one of partition. Some of the solvents recommended are, in their substantially anhydrous forms, solvents for the unsulphonated or low SO<sub>3</sub> fractions as well as possessing solvent powers for the fraction having a high SO<sub>3</sub>. It appears, however, that the solvents in the presence of moisture have a greater affinity for the high SO<sub>3</sub> fraction than that of the low SO<sub>3</sub> fraction, thus giving rise to the unexpected results. In view of this condition, the aforementioned terms are used to describe the partitioning action of the solvent with respect to the high and low SO<sub>3</sub> fractions.

For a fuller understanding of the nature and objects of the invention, reference should be had to the following examples which are given merely

to further illustrate the invention and which are not to be construed in a limiting sense.

#### Example I

300 grams of sulphonated olive oil (neutralized by an alkaline wash and containing 30% water) containing 9.8% organically combined SO<sub>3</sub> was agitated with 300 cc. of acetone and allowed to stand until separation into two layers was caused to take place. Upon separation of the layers and removal of solvent by distillation, 108 grams of extracted oil (upper layer) with an SO<sub>3</sub> content of 12.3% and 178 grams of residual oil (lower layer) with an SO<sub>3</sub> content of 8.2% resulted.

#### Example II

By carrying out the same procedure as outlined in Example I using 600 cc. of acetone (twice the amount), the following yield was obtained: 149 grams of extracted oil with an SO<sub>3</sub> content of 11.3% and 113 grams of residual oil having an SO<sub>3</sub> content of 7.1%.

From a comparison of the above examples, it may be noted that the use of a smaller quantity of solvent, as in Example I, gave a smaller yield but of a higher SO<sub>3</sub> value than that obtained by using a larger quantity of solvent (as in Example II).

#### Example III

380 grams of sulphonated olive oil (about 30% moisture) containing 8.8% organically combined SO<sub>3</sub> was agitated with 380 grams of methyl alcohol. After separation of the two layers which resulted on standing and removal of the solvent, the oil in the upper layer had an organically combined content of 13.9% and the oil in the lower layer showed an SO<sub>3</sub> content of 6.4%.

#### Example IV

In carrying out the same process outlined in Example III, using ethyl alcohol in lieu of methyl alcohol, the oil in the upper layer showed an organically combined SO<sub>3</sub> value of 10.4%.

The expression "sulphonated naturally occurring fatty materials" is employed in the appended claims to connote the water-soluble salts of sulphated fatty acids, fatty triglycerides and fatty waxes. Likewise the expression "sulphonated" is used to define the water-soluble salts of the sulphuric acid esters produced on sulphonation of fatty materials.

Since certain changes may be made in carrying out the above process without departing from the scope of the invention, it is intended that all matter contained in the above description shall be interpreted as illustrative and not in a limiting sense.

It is also to be understood that the following claims are intended to cover all the generic and specific features of the invention herein described, and all statements of the scope of the invention, which as a matter of language might be said to fall therebetween.

Having described my invention, what I claim as new and desire to secure by Letters Patent is:

1. In a process for increasing the SO<sub>3</sub> content of sulphonated naturally occurring fatty materials, the step which comprises subjecting the sulphonated material to extraction with an organic, water-miscible solvent, in an amount at least equal to the volume of the sulphonated fatty material.

2. A process for increasing the SO<sub>3</sub> content of sulphonated naturally occurring fatty mate-

rials which comprises mixing such sulphonated materials with an organic water-miscible solvent, allowing the mixture to settle whereby two layers form, one containing dissolved sulphonated material and the other containing unsulphonated material and separating the respective layers.

3. The process in accordance with claim 1 wherein the solvent used comprises a substance selected from the group consisting of low molecular weight alcohols and ketones.

4. In a process for increasing the  $\text{SO}_3$  content of sulphonated triglycerides, the step which comprises subjecting a sulphonated triglyceride to extraction with a water-miscible organic solvent.

5. In a process for increasing the  $\text{SO}_3$  content of sulphonated olive oil, the step which comprises subjecting a sulphonated olive oil to extraction with a water-miscible organic solvent.

6. In a process for increasing the  $\text{SO}_3$  content of sulphonated cod oil, the step which comprises subjecting a sulphonated cod oil to extraction with a water-miscible organic solvent.

7. In a process for increasing the  $\text{SO}_3$  content of sulphonated cottonseed oil, the step which comprises subjecting a sulphonated cotton seed oil to extraction with a water-miscible organic solvent.

8. In a process for increasing the  $\text{SO}_3$  content of sulphonated triglycerides, the step which comprises subjecting a sulphonated triglyceride to extraction with a water-miscible organic solvent selected from the group consisting of low molecular weight alcohols and ketones.

9. In a process for increasing the  $\text{SO}_3$  content of sulphonated olive oil, the step which comprises subjecting a sulphonated olive oil to extraction with a water-miscible organic solvent selected from the group consisting of low molecular weight alcohols and ketones.

10. In a process for increasing the  $\text{SO}_3$  content

of sulphonated cod oil, the step which comprises subjecting a sulphonated cod oil to extraction with a water-miscible organic solvent selected from the group consisting of low molecular weight alcohols and ketones.

11. In a process for increasing the  $\text{SO}_3$  content of sulphonated cottonseed oil, the step which comprises subjecting a sulphonated cottonseed oil to extraction with a water-miscible organic solvent selected from the group consisting of low molecular weight alcohols and ketones.

12. In a process for increasing the  $\text{SO}_3$  content of sulphonated olive oil, the steps which comprise mixing the sulphonated olive oil with a low molecular weight ketone, permitting the mixture to settle whereby two layers form, one containing sulphonated material dissolved in said low molecular weight ketone and the other containing unsulphonated material, and separating the respective layers.

13. In a process for increasing the  $\text{SO}_3$  content of sulphonated cod oil, the steps which comprise mixing the sulphonated cod oil with a low molecular weight ketone, permitting the mixture to settle whereby two layers form, one containing sulphonated material dissolved in said low molecular weight ketone and the other containing unsulphonated material, and separating the respective layers.

14. In a process for increasing the  $\text{SO}_3$  content of sulphonated cottonseed oil, the steps which comprise mixing the sulphonated cottonseed oil with a low molecular weight ketone, permitting the mixture to settle whereby two layers form, one containing sulphonated material dissolved in said low molecular weight ketone and the other containing unsulphonated material, and separating the respective layers.

BERNARD A. DOMBROW.